

## UNITED STATES PATENT OFFICE

SHERWIN P. LOWE, OF DENVER, COLORADO, ASSIGNOR TO R. H. CHANNING, AGENT, OF DENVER, COLORADO

## FLOTATION PROCESS

No Drawing.

Application filed March 26, 1928. Serial No. 264,965.

My invention relates to the concentration of ores by oil flotation, and has particularly in view the obtaining of higher grade concentrates from complex ores containing copper or lead and zinc. In the flotation concentration of such ores, soluble salts such as copper sulphate or ferrous sulphate, are often present, either in the water, in the ore, or released during grinding or the preparation of the ore. These soluble salts interfere with the proper selective action of the froths. This condition can be partially overcome by the addition of lime, but may be almost entirely overcome by the addition of zinc oxide in suitable quantities—which acts as a precipitant for the objectionable salts—in addition to the other reagents commonly used in flotation.

An example of the effect of zinc oxide is as follows:

An ore assaying 1.9% Cu, 4.6% Zn, and 30% iron was ground with 4 lbs. CaO per ton and one part of water, and these placed in a flotation machine and .1 lb. pine oil and .1 lb. zanthate, per ton of ore, was added, and a copper concentrate was removed. The results were as follows:

|                 | Per cent Cu | Per cent Zn |
|-----------------|-------------|-------------|
| Cu concentrates | 17.0        | 5.3         |
| Tailings        | .3          | 4.55        |

The same ore was treated in the same manner, except that 2 lbs., per ton of ore, of zinc oxide was added to the ore before grinding, the results were:

|                 | Per cent Cu | Per cent Zn |
|-----------------|-------------|-------------|
| Cu concentrates | 20.0        | 3.8         |
| Tailings        | .25         | 4.65        |

## What I claim is:

1. The process of concentrating ores by froth flotation comprising the step of adding zinc oxide in addition to other well known oils and reagents, to the pulp to obtain higher grade concentrates.
2. The process of concentrating ores by froth flotation comprising the step of adding zinc oxide, in addition to other well known oils and reagents, to the pulp to overcome the effect of interfering soluble salts and to obtain higher grade concentrate.

3. The process of concentrating complex ores containing zinc and one of the metals of the group comprising copper and lead, by froth flotation, comprising the step of adding zinc oxide, in addition to other well known oils and reagents, to the pulp to decompose interfering mineral salts and to increase the efficiency of the flotation agent.

4. The process of concentrating ores by froth flotation comprising the step of adding a small quantity of zinc oxide, in addition to other well known oils and reagents, to the pulp to obtain higher grade concentrates by overcoming the effect of soluble salts.

5. The process of concentrating complex ores containing zinc and one of the metals of the group comprising copper and lead by froth flotation, comprising the step of adding approximately 2 lbs. of zinc oxide, in addition to other well known oils and reagents, to the pulp to decompose the soluble salts and to increase the efficiency of the flotation agent.

In testimony whereof, I affix my signature.

SHERWIN P. LOWE.